

## UNITED STATES PATENT OFFICE

ALBERT A. SOMERVILLE, OF FLUSHING, NEW YORK, ASSIGNOR OF TWO-THIRDS TO  
R. T. VANDERBILT COMPANY, INCORPORATED, OF NEW YORK, N. Y., A CORPORA-  
TION OF NEW YORK

## HEAT TREATMENT OF METALS

No Drawing.

Application filed July 15, 1926. Serial No. 122,729.

This invention relates to improvements in the heat treatment of metals and includes improved heat treatment baths and also improvements in the method of heat treatment 5 of the metals.

More particularly, the invention relates to improvement in oil baths for the heat treatment of metals and the heat treatment of the metals therewith.

10 When oil baths are used for tempering or heat treating metals and alloys, the bath may be maintained at high temperatures for prolonged periods of time with resulting tendency of the oil baths to change in composition and to deteriorate.

According to the present invention, the oil baths have combined therewith a stabilizing ingredient, or stabilizing ingredients, whereby the deterioration of the oil composition 20 is prevented or reduced or its rate of deterioration more or less regulated and controlled so that it will have improved stability and resistance to objectionable deterioration.

According to the present invention, I add 25 to and incorporate with the oil bath used for the tempering or the heat treatment of the metal, a small amount of a condensation product of a carbonyl derivative (aldehydes or ketones) with a nitrogenous base such as 30 ammonia and amines, which condensation product serves as a stabilizing agent to retard or prevent or regulate objectionable deterioration of the composition.

The oil compositions which are employed 35 in the present invention include oil compositions such as are commonly used for oil baths in tempering and heat treatment of metal. The oil baths may be, for example, such as are employed to heat metals up to the proper 40 temperature, for example, a temperature of around 500° F., or they may be oil compositions such as are used for quenching heated metals in which case the temperature of the bath may be kept at or below 100° F., or at 45 a regulated higher temperature, except for local overheating caused when the highly heated metal is introduced into the oil bath. For the latter purpose, mineral oils, animal oils, vegetable oils, and mixtures of these are 50 used, cotton seed oil being a preferred oil

among the fatty oils, because of the tendency of oils like linseed oil to become gummy and of the animal and fish oils to become rancid or give off offensive odors. The invention is of particular value with mineral oils, or mixtures containing mineral oils, suitable for use for tempering or heat treatment of metals.

According to the present invention, such tempering or heat treatment oil compositions or baths have incorporated therewith a small amount of a condensation product of an aldehyde or ketone with a nitrogenous base. The condensation product should be soluble or miscible with the oils so they are 60 intimately distributed throughout the composition. They may be added directly to the composition or to certain ingredients of the composition, or they may be first dissolved in a solvent such as benzol and added in that 65 form with subsequent heating of the mixture to remove the benzol.

The amount of the condensation product which it is necessary to add is small. In general, a few percent at most will suffice, and as little as a fraction of a percent may be 70 sufficient, e. g., 0.5% to 1%.

The invention will be further illustrated by the following specific examples, but it is intended and will be understood that the invention is illustrated thereby but is not limited thereto.

A mineral oil composition of a consistency and character suitable for use for tempering or heat treatment of metals, has added thereto about 1% of a condensation product of acet-aldehyde and aniline. The admixture of the condensation product with the oil can be promoted by dissolving the condensation product first in benzol, then admixing the benzol solution with the oil and if need be, driving off the benzol, although it will ordinarily be removed during the subsequent use of the composition so that separate treatment for removal may be unnecessary. The resulting oil composition will have improved properties when used as a tempering or heat treatment bath.

In a similar manner, a mixed mineral oil and vegetable oil composition (e. g. containing cotton seed oil) may have added thereto a

55

60

65

70

75

80

85

90

95

100

small amount, for example, 1/2% to 2%, of the condensation product above referred to.

In a similar manner, other tempering or heat treatment oil baths may have a small amount of one or another of the condensation product added thereto and incorporated therewith, thus imparting to the composition improved stability and resistance to deterioration.

10 Instead of using the condensation product of acetaldehyde and aniline, the condensation product of aldol and alpha-naphthylamine can be similarly used, or other condensation products of aldehydes, such as formaldehyde, acetaldehyde, benzaldehyde, butyraldehyde, furfuraldehyde, aldol, etc., with amines, both aliphatic and aromatic, e. g., anilin, alpha or beta naphthylamine, or with ammonia, etc. Examples of such condensation products, in 20 addition to those above mentioned, are the condensation product of formaldehyde with aniline, the condensation product of acetaldehyde with aniline (both the acid and the neutral condensate), the condensation product of 25 acetaldehyde with ortho or para-toluidine, etc., the condensation product of furfuraldehyde with ammonia or with anilin or ortho-toluidine, etc. The condensation product of certain aldehydes and amines can be carried 30 out either with or without an acid condensing agent, and the condensation product may be different in the different cases. When an acid condensing agent is used, it may be considered that the amine is used in the form of its salt, 35 but when after the condensation the product is neutralized with caustic soda, the salt forming group will be removed. The condensation product may nevertheless in such case be different from that produced when no acid 40 is used. Various amines, both aromatic and aliphatic, can be used for the condensation, as well as various aldehydes.

In a similar manner, condensation products of ketones and nitrogenous bases can be 45 used, for example, condensation products of acetone with ammonia, etc.

In using the new stabilized oil compositions, they may be heated to the temperature at which such baths are commonly heated for 50 tempering or heat treating purposes, and the metals can be immersed therein and heated thereby, or in the case of highly heated metals, may be cooled and quenched thereby. The presence in the oil bath of the stabilizing material will impart thereto improved stability 55 against deterioration by atmospheric oxidation, as well as other improved properties, thereby prolonging the useful life of the bath before it needs to be discarded and replaced.

60 I claim:

1. Improved heat treatment baths for the tempering or heat treatment of metals, comprising oils having combined therewith a small amount of a condensation product of a 65 carbonyl derivative with a nitrogenous base.

2. Improved heat treatment baths for the tempering or heat treatment of metals, comprising oils having combined therewith a small amount of a condensation product of an aldehyde with a nitrogenous base.

3. Improved heat treatment baths for the tempering or heat treatment of metals, comprising oils having combined therewith a small amount of a condensation product of an aldehyde with an amine.

4. The improvement in the tempering or heat treatment of metals, which comprises immersing the metal in an oil composition and reducing objectionable decomposition of said composition and prolonging its useful life by incorporating therein a small amount of a condensation product of a nitrogenous base with a carbonyl compound.

5. The improvement in the tempering or heat treatment of metals, which comprises immersing the metal in an oil composition and reducing objectionable decomposition of said composition and prolonging its useful life by incorporating therein a small amount of a condensation product of a nitrogenous base with a carbonyl compound.

6. The improvement in the tempering or heat treatment of metals, which comprises immersing the metal in an oil composition and reducing objectionable decomposition of said composition and prolonging its useful life by incorporating therein a small amount of a condensation product of a nitrogenous base with an aldehyde.

In testimony whereof I affix my signature. 100  
ALBERT A. SOMERVILLE.

105

110

115

120

125

130